

1,415,094.

D. B. JONES,  
ORE-BRIQUETTE.  
APPLICATION FILED JUNE 3, 1918.

Patented May 9, 1922.



Witness:

*Geo. S. Johnson*

Inventor

*David B. Jones*  
By *Acton B. Jones*

# UNITED STATES PATENT OFFICE.

DAVID B. JONES, OF CHICAGO, ILLINOIS.

## ORE BRIQUETTE.

1,415,094.

Specification of Letters Patent. Patented May 9, 1922.

Original application filed June 22, 1914, Serial No. 846,466. Divided and this application filed June 3, 1918. Serial No. 237,862.

To all whom it may concern:

Be it known that I, DAVID B. JONES, a citizen of the United States, residing in Chicago, in the county of Cook and State of Illinois, have invented certain new and useful Improvements in Ore Briquettes, of which the following is a specification, reference being had to the accompanying drawings, forming a part thereof.

10 My invention is more specifically concerned with the production of zinc, and in the following specification is described in connection therewith, but it will be understood that in some respects, and particularly 15 in its broader aspects, it is also applicable to other ores. It relates to the form and also to the construction and composition of briquettes by reason of which they are particularly adapted for use in a certain process 20 forming the subject-matter of a Patent No. 1,292,330, granted to me January 21, 1919, on an application of which the present application is a division, and in a new and improved type of furnace shown and described 25 but not claimed in said patent, and forming the subject-matter of another application No. 237,867 of even date herewith.

Briefly described said furnace comprises a heating chamber in the hearth, of which 30 are arranged or formed inclined guides leading from the charging end of the furnace to the exit end thereof, along which the briquettes are fed by gravity, and in the practice of said process the briquettes, which are 35 composed largely of the ore and a reducing material, are subjected to a temperature which distills off the zinc, and surrounded by an oxidizing atmosphere by which the zinc vapor given off is converted into the 40 oxide, carbonate or both, and collected as such. My improved briquette is rounded, and in the preferred form spherical, which permits it to roll along said guides no matter how placed thereon, the period of its 45 transit through the furnace being sufficiently extended and the temperature of the furnace such as to substantially drive off all the zinc contained in the briquette without, however, driving off any lead or silver which the ore 50 may contain. The spherical form of briquette also has the advantage that it con- 55 ducts to equal heating and expansion throughout so that no such strains are set up during the heating as would tend to split up and disintegrate the briquette. In order to make a substantial briquette which will

stand up under the treatment to which it is subjected and not readily disintegrate, I employ with the mixture of ore a reducing agent or a binder preferably of inorganic 60 matter, and coat the briquette with a relatively thin layer of refractory material which is sufficiently pervious to permit the escape of the zinc vapors therethrough.

In the accompanying drawings Fig. 1 is 65 a vertical longitudinal section of a furnace designed for the treatment of my improved briquettes and as covered in the aforesaid application of even date; Fig. 2 is a vertical transverse section thereof on the line 2—2 of 70 Fig. 1; Fig. 3 an inclined transverse section parallel to the hearth of the furnace on the line 3—3 of Fig. 1; and Fig. 4 is a cross section illustrating the improved briquette.

Referring first to Figs. 1, 2 and 3, the 75 furnace comprises the usual side walls and roof arranged however at an incline, but the hearth or bottom of the furnace is composed of longitudinal extending piers or walls A spaced slightly apart and supported with 80 respect to each other by the interposed blocks or bricks a. The upper edges of the walls are chamfered or cut away as shown in Fig. 2, to form between each pair of adjacent walls a track or runway down which the 85 briquettes B travel. In the particular furnace shown there are nine of these runways, but obviously this number might be increased or diminished according to the capacity of furnace desired. At the upper or front end 90 of the furnace an opening or doorway C is provided in register with each track or runway, and is closed by a suitable door, and at the lower or discharge end of the furnace a door D normally closes the opening opposite 95 each track. At suitable intervals to provide the proper length of treatment for each briquette a new briquette is inserted at the upper end of each track or runway, and the end briquette at the lower end of such runway permitted to drop into a storage chamber E from which the briquettes may be removed as they accumulate. The furnace is heated by means of gas and air, the air being 100 conveyed to transverse chambers X extending transversely of the piers or walls forming the hearth by means of perforated pipes F<sup>2</sup> extending from a longitudinal pipe F' leading from the blower F and gas being supplied to said transverse chambers by 105 transverse perforated pipes G<sup>2</sup> connected to a longitudinal main G' leading to some suit- 110

able supply of fuel gas. The flame and heated products of combustion not only heat the longitudinal pier walls, but rising between and about the briquettes B heat 5 them to the desired temperature. Preferably the heat from the briquettes B in the chamber E is used to pre-heat the air used in connection with this furnace, and for this purpose the fan F supplying air is connected 10 to the chamber E and the longitudinal pipe F' likewise opens thereinto so that the air previous to its passage to the burner pipes is heated to a considerable temperature. The zinc distilled from the briquettes may be collected 15 in any suitable manner, but preferably I provide an additional supply of air for oxidizing it and collect it in the form of the oxide, the air being supplied to the chamber H above the briquettes through a branch 20 pipe E' connecting said chamber and storage chamber E, said pipe being controlled by the valve or damper E<sup>2</sup>.

Referring now to Fig. 4, the interior of the briquette shown at B' is composed of a 25 mixture of the ore being treated, a sufficient quantity or proportion of reducing material and a binder. The reducing material preferably employed is pulverized coal and the binder is preferably an inorganic material 30 such as bauxite. The reducing material ordinarily being somewhat in excess of that theoretically required to reduce the zinc ore contained in the mass and the binder being of sufficient quantity when mixed with water 35 or other liquid to firmly unite the particles of ore and reducing material. After the mixture above described has been made the briquettes are formed, preferably, in molds under very high pressure, and are 40 then permitted to dry until they are sufficiently rigid for further treatment. They are then covered with a slip of fire clay or a light refractory material by dipping or otherwise, after which they are slowly heated 45 and dried to drive off all the contained moisture preparatory to charging the briquettes into the furnace. It will be found that the relative amounts of ore reducing agent and binder will vary with the particular ore 50 used, and the best proportions may be readily determined by experiment. Instead of water alone a solution of common salt may be employed for bringing the materials into plastic form and for making a slip or 55 grout with which the briquettes are covered, the salt remaining in the briquettes after the water has been driven off and acting in a measure as a flux. Any form of press may be used which will furnish the desired pressure 60 to produce great compactness and solidity in the briquettes, and any form of kiln may be used for drying the briquettes,

though preferably they are dried quite slowly and at a temperature of about 220 degrees Fahrenheit, which temperature ordinarily twenty-four hours or longer is required to complete the drying operation. The drying may be done either before or after the application of the coating of fire clay, but if done mainly before such application it is preferable to again dry the briquettes sufficiently to drive off the moisture imparted by the application of the fire clay. 70

In the furnace the briquettes are gradually raised to a temperature at which the 75 zinc oxide or other zinc compound contained in the briquettes is reduced by the powdered coal or other reducing agent and volatilized. But the zinc vapors coming into the oxidizing atmosphere maintained in the furnace 80 are converted into the oxide and the fumes passing off through the conduit I may be collected in any of the devices commonly employed in pigment furnaces for such purposes. 85

As many zinc ores also contain compounds of lead or silver or both it is preferable to keep the temperature of the furnace below that at which these metals are volatilized, and after the briquettes have been substantially deprived of their zinc content they 90 may be given further treatment in ordinary vertical furnaces or the like for recovering the other valuable metal contents thereof. 95

Obviously certain advantages of my improved briquette may be obtained in furnaces other than those of the type just described, the superior resistance of the briquettes due to their composition, construction and form being valuable in many 100 of the old and well-known types of furnace, and it is not absolutely essential to feeding the brick through the furnace by gravity that they be spherical so long as they are substantially circular in cross-section though 105 if they are not spherical care must be taken that they be so placed in the guides or runways as to roll down the same when the lowermost briquettes are withdrawn. 110

I claim:

1. A briquette composed of zinc ore, a reducing agent and a binder of bauxite. 110
2. A briquette composed of zinc ore, a reducing agent, a plastic inorganic binder and common salt. 115
3. A briquette comprising a mixture of zinc ore, reducing material, and a binder, and having a slip coating of pervious highly refractory material thereon.
4. A briquette comprising a mixture of zinc ore, reducing material and a binder, having a coating of fire clay thereon. 120

DAVID B. JONES.